

# UNITED STATES PATENT OFFICE.

PAUL BUNET, OF PARIS, FRANCE, ASSIGNOR TO SOCIETE GENERALE DES NITRURES, OF PARIS, FRANCE, A CORPORATION OF FRANCE.

## PROCESS FOR THE FIXATION OF NITROGEN BY MEANS OF FERRO-ALUMINIUM.

1,196,657.

Specification of Letters Patent. Patented Aug. 29, 1916.

No Drawing.

Application filed April 3, 1915. Serial No. 19,062.

*To all whom it may concern:*

Be it known that I, PAUL BUNET, a citizen of the Republic of France, and a resident of 12 Rue Roqueline, Paris, France, have invented a new and useful Improvement in Processes for the Fixation of Nitrogen by Means of Ferro-Aluminium, of which the following is a specification.

In the specifications of U. S. patent applications filed December 20, 1913, under Serial No. 807,915, filed December 23, 1913, under Serial No. 808,478, and filed November 18, 1914, under Serial Number 872,837, various processes for the fixation of nitrogen

15 by means of ferro-aluminium are described.

The surprising fact has been ascertained that, in these various processes, when to the ferro-aluminium a certain quantity of calcium carbid is added, the fixation of the 20 nitrogen is considerably hastened and increased in such a way that the operator can fairly rapidly reach and even exceed the theoretical proportion of nitrogen which the aluminium contained in the ferro-alu-

25 minium is capable of fixing.

In the preparation of the ferro-aluminium starting from bauxite, which generally con-

tains a little lime, it is possible that there may be formed incidentally, a little calcium carbid, but even in the case where it is so formed the quantity thus produced is less than the quantity which should be added to obtain the most favorable result.

By way of example, if a mixture of 200 kilograms ferro-aluminium (42 per cent. of aluminium) with 40 kilograms of calcium carbid (54 per cent. of  $\text{CaC}_2$ ) be treated with heat in a current of nitrogen, a product can be obtained, containing as much as 44.75 kilograms of nitrogen, which is more than the aluminium content alone is theoretically capable of fixing.

I claim as my invention:—

In the processes of fixation of nitrogen on ferro-aluminium by subjecting a mass containing ferro-aluminium to a current of nitrogen, adding calcium carbid to said mass.

In testimony whereof I have signed my name to this specification, in the presence of two subscribing witnesses.

PAUL BUNET.

Witnesses:

CHARLES DORUO,  
DE W. C. POOLE, Jr.

Copies of this patent may be obtained for five cents each, by addressing the "Commissioner of Patents, Washington, D. C."